

Dec. 10, 1929.

G. L. BENNETT

1,739,056

METHOD OF FINISHING SHEET METAL TILING

Filed Sept. 15, 1928

*Fig. 1.*



*Fig. 2.*



*Fig. 3.*



*Fig. 4.*



*Fig. 5.*



*Fig. 6.*



George L Bennett

INVENTOR

BY Frank P. Wentworth  
his ATTORNEY.

## UNITED STATES PATENT OFFICE

GEORGE L. BENNETT, OF CLEVELAND HEIGHTS, OHIO

## METHOD OF FINISHING SHEET-METAL TILING

Application filed September 15, 1928. Serial No. 306,161.

The invention relates to a method of finishing sheet metal tiling, and more particularly to a method of finishing the edges of large sheets of tiling when producing, or when fitting same to a wall space, so as to permit adjacent sheets to be accurately fitted when mounting them upon the wall of a room while preserving continuity of the vitreous enamel surface and avoiding subsequent deterioration of the metal at the butt joints between such sheets through erosion of the metal, which would result in possible discoloration at the joint, or the breaking down of the bond between the enamel and the metal sheet, and consequent chipping of the enamel.

Sheet metal tiling of the character with which the method of my invention is to be used, consists of ordinary thin gauge rolled metal, such as steel, having a vitreous enamel applied to at least that face thereof to be exposed within a room, the finished face of the sheet being provided with a design, or being in continuous color, as desired.

These sheets are of a length to extend substantially between the ceiling of a room and the floor, and are secured in place in any desired manner. The detailed construction of such tiling sheets and the manner of mounting same forms no part of the present invention, which is applicable to the finishing operation of such sheets irrespective of such details.

In the enamel surfacing of sheet metal, there is, during the baking operation, a shrinkage of the enamel away from the opposite edges of the sheet, or adjacent the sharp edge of the metal. This shrinkage is sufficient to produce defects in the enamel surface along this edge, and present blemishes at the meeting lines of different sheets. It is impossible to correct this condition by enamelling the edges of the sheet, since the enamel will shrink away from the sharp edge of the metal, and a curvature at this point will prevent a close fitting of adjoining tiling sheets.

Furthermore, while such tile sheets may be made to standard dimensions, there is always a necessity for cutting and fitting such sheets in adapting them to rooms of different dimensions, to angles in a room and about openings.

With such tiling it is impossible to bend same without disrupting the enamel surface. Consequently, fitting requiring variation in the dimensions of the sheet, and at times, at an angle of a room, necessitates the cutting of the sheet and, as in producing the sheets, blemishes adjacent the edge of a sheet and conditions resulting in erosion of the metal at the edge must be avoided.

Therefore, in cutting and fitting sheets, such sheets should have the same edge finish as when producing sheets of standard size.

In trimming or cutting sheet metal tiling having a decorative surface of vitreous enamel, the various tools and implements commonly used in the cutting of sheet metal cannot be resorted to, because such tools and implements will chip the enamel from the surface adjacent the cut and thus produce blemishes in the finish along abutting edges of adjoining sheets. Furthermore, if such methods are resorted to, the edge of the metal sheet is subject to erosion from oxidation or other causes, which in time extends beneath the enamel surface and destroys the bond between the enamel and the sheet metal.

With the above conditions in mind, I have devised a method of finishing vitreous enamel coated sheet metal tiling by which any desired portion adjacent the edge of a tiling sheet may be separated from the body of the sheet without chipping or otherwise mutilating the decorated face of the sheet, and then so protecting the edge of the metal at the cut as to preclude possibility of erosion affecting the metal at the line of joinder between same and the enamel surfacing.

By the method of my invention, sharp clean edges of the tiling sheets are assured, and the healing or protecting medium at the edge is such as to avoid the presence of any appreciable seam along the abutting edges of adjoining tiling sheets as a result of the presence of the material used for thus healing the edge.

The invention consists primarily in a method of finishing sheet metal tiling, embodying therein the separation of one portion of an enamel coated metal sheet from another portion thereof by abrasion, and subsequently coating the exposed edge of the body of the

sheet with a non-corrosive material; and in such other novel steps and practices, as are hereinafter set forth and described, and more particularly pointed out in the claims hereto appended.

5 Referring to the drawings,

Figs. 1, 2 and 3 illustrate in side elevations, front elevation and in plan the step of separating a vitreous enamel coated metal tiling sheet;

10 Figs. 4 and 5 show in side elevation and in plan the healing of the cut resulting from the first step of the method; and

15 Fig. 6 shows in section a fragmentary portion of one edge of the finished sheet.

Like letters refer to like parts throughout the several views.

In the embodiment of the invention as illustrated in the accompanying drawings, one 20 portion of the vitreous coated sheet metal tile strip is shown at *a*, and the portion thereof to be removed, at *a'*. In order to separate the portion *a'* from the portion *a*, I make a line of division between the part *a* and the part *a'* 25 by abrasion, utilizing some tool such as an emery or carborundum wheel which will effectively cut the vitreous enamel surface *b* of the sheet as well as the metal portion *c* thereof, without chipping or cracking the 30 enamel. The cut is at substantially right angles to the surface of the sheet so as to produce a flat surface at the edge which will squarely abut against a similar surface upon an adjoining tiling sheet, in mounting same 35 upon a wall.

When the part *a'* has been thus separated from the part *a* of the tiling sheet, I apply 40 a protective surfacing *d*, of non-corrosive material, to this edge to prevent erosion, particularly the line of junction between the 45 metal portion of the sheet and its enamelled surface. This protecting coating or healing medium for the cut is preferably a thin coating of solder applied to the edge of the sheet following the application of a suitable flux.

In order to simplify the healing step and secure greater uniformity, I preferably employ a mechanism such as is shown in Figs. 4 and 5, by which, with a continuing movement 50 of the sheet, every portion thereof is successively brought into engaging relation with a device for applying the flux thereto, and with a soldering wheel immersed in molten solder and brought to the desired temperature.

55 While the solder will readily adhere to, and form a protective coating for, the edge of the metal portion of the sheet, it will not adhere to the enamel surfacing. Nor will the temperature at which the solder is applied have any effect upon this enamel surfacing.

60 While the tools employed in carrying on the method are immaterial thereto, I have shown certain tools and appliances in the accompanying drawings and will describe same

herein. As shown in Figs. 1 to 3, I employ a narrow abrasive wheel *e*, driven at high speed by a motor *f* and carried by a channelled base *g*, the sides of which are adapted to engage the opposite sides of a straight edge *h*, which, 70 after being laid upon the portion *a* of the sheet, is secured to a bench *i* having a slot *i'* therein. The portion *a* rests upon this bench and extends across said slot *i'*. The straight edge is secured to the bench in a position to 75 bring the abrasive wheel *e* in the proper position in relation to a selected line of severance between the portions *a*—*a'* of the sheet. The base *g* is provided with a gauge finger *g'* which may be alined with a gauge marking 80 *a*—*a'* upon the tiling sheet.

In Figs. 4 and 5 I have shown a desirable form of device for applying the non-corrosive facing to the cut edge of the portion *a*. This consists of a tank *j* for flux, having therein a 85 flanged roller *j'*. Adjacent this tank *j* is a solder pot *k*, having a flanged roller *k'* to pick up solder from the pot *k* and carry it to a point of application to the edge of the sheet portion *a*. Adjacent the pot *k* and the roller *k'* is a suitable heating device *k*<sup>2</sup> directing the flame against the pot *k* and the roller *k'* so as to maintain these at the desired temperature. The tank *j* and the pot *k* and their appurtenances are supported by a bench *m*.

90 In producing enamel surface tiling sheets of standard dimensions, it is necessary to trim only the side edges of the sheet, since ordinarily the trim of the room will cover the end edges. If desired, however, each 100 sheet may be trimmed about all edges.

In the finishing operation, the tiling sheet is secured in position, and the abrading wheel *e* is used to remove a narrow width of the sheet at the line of demarcation of the portion *a* and the portion *a'* thereof, the action of the wheel being not only to grind away the metal and its enamel surface, but to produce a ground finish at the edge of the portion *a*. The abrasive action of said wheel will not 105 chip the vitreous enamel so that upon the removal of the portion *a'*, the decoration afforded by the enamel surfacing *b* will extend to the very edge of the sheet without blemishes of any kind due to shrinkage of the enamel in baking or to the cutting of the portion *a'* from the sheet. The opposite edges of the sheet will be similarly trimmed, and, if desired, the end edges may also be 110 trimmed, although as stated this is unnecessary if the trim of the room is such as to cover any blemishes or defects at these edges.

115 After a portion *a'* has been removed from a tiling sheet, the remaining portion *a* is passed edgewise in engaging relation with the rollers *j'* and *k'*, the former of which will apply flux to the ground edge of the portion *a*, and the latter of which will apply solder thereto in a thin coat by reason of the pressure relation between the edge of the 120

sheet and the roller *k'*, which coat will be very thin but of substantially uniform thickness.

It is of primary importance to have a lamina of the solder or other non-corrosive substance upon the edge of the sheet metal *c* extend to the juncture of the surface of said sheet and the enamel surfacing *b*, in order to prevent erosion at the line of demarcation between said sheet *c* and said coating *d*. Otherwise such erosion would, in time, result in the flecking or chipping of the enamel adjacent the edge of the sheet. If necessary, the solder applied to the edge of the sheet metal seam may be smoothed down by an ordinary hand soldering iron.

A portion of the finished product upon a greatly exaggerated scale is shown in Fig. 6.

By finishing tiling sheets by the method 20 of my invention, each sheet of standard dimensions will have smooth sharp edges ground to a fine finish along a perfectly straight line, so that when mounting the sheets upon the wall of a room, the edges 25 of each sheet will squarely abut against the edges of adjoining sheets. The decorative vitreous enamel surface will extend to the extreme edge of each sheet, since the solder coating will not be of a thickness to result 30 in a discernible seam.

The edge of the metallic portion *c* of the tiling sheet will be protected against erosive action of the elements after the insulation of the sheet, as a result of the healing of the cut 35 by the solder or other non-corrosive surfacing material applied to this edge.

While above I have referred more particularly to the finishing method as applied to sheets of standard dimensions, it is obvious 40 that the same methods may be employed in producing, from a standard size sheet, smaller or narrower sheets when such is required for the proper mounting of sheet tiling upon the walls of a room.

45 It is not my intention to limit the invention to the particular tools or appliances used in carrying on the method of my invention, nor to the use of solder as the healing material or edge stratum of the sheets. The mechanisms described herein are merely illustrative of tools and appliances which may be used in the expeditious practice of the invention.

Having described the invention, what I 55 claim as new and desire to have protected by Letters Patent, is:—

1. A method of finishing sheet metal tiling, embodying therein the separation of one portion of an enamel coated metal sheet from another portion thereof by abrasion, and subsequently coating the exposed edge of the body of the sheet with a non-corrosive material.

2. A method of finishing sheet metal tiling, 65 embodying therein the separation of one por-

tion of an enamel coated metal sheet from another portion thereof by abrasion, and subsequently applying a thin coating of solder to the exposed edge of the metal portion of the sheet.

3. A method of finishing sheet metal tiling, 70 embodying therein the separation of one portion of an enamel coated metal sheet from another portion thereof by simultaneously cutting the enamel surface and the sheet metal by means of an abrading medium, whereby a flat ground finish is also produced at the edges of the cut, and subsequently coating the exposed edge of the metal portion of the sheet with a non-corrosive material.

4. A method of finishing sheet metal tiling, 75 embodying therein the separation of one portion of an enamel coated metal sheet from another portion thereof by simultaneously cutting the enamel surface and the sheet metal by means of an abrading medium, whereby a flat ground finish is also produced at the edges of the cut, and subsequently applying 80 a thin stratum of a non-corrosive metal to the edge of the metal portion of the sheet.

5. A method of finishing sheet metal tiling, 85 embodying therein the separation of one portion of an enamel coated metal sheet from another portion thereof by simultaneously cutting the enamel surface and the sheet metal by means of an abrading medium, whereby a flat ground finish is also produced at the edges of the cut, and subsequently applying 90 a thin coating of solder to the edge of the metal portion of the sheet.

In witness whereof I have hereunto affixed my signature this 12th day of September, 1928.

GEORGE L. BENNETT. 105

110

115

120

125

130